

# United States Patent

Hu

[15] 3,676,346

[45] July 11, 1972

[54] **LUBRICATING OIL COMPOSITIONS  
CONTAINING IMPROVED SLUDGE  
INHIBITING ADDITIVES**

[72] Inventor: **Shih-En Hu**, Westfield, N.J.  
[73] Assignee: **Esso Research and Engineering Company**  
[22] Filed: **Feb. 19, 1970**  
[21] Appl. No.: **12,869**

[52] U.S. Cl.....252/47.5, 252/45, 252/48.6  
[51] Int. Cl.....C10m 1/38  
[58] Field of Search.....252/47.5, 51.5, 45, 48.6, 406

[56] **References Cited**

UNITED STATES PATENTS

|           |         |                    |            |
|-----------|---------|--------------------|------------|
| 3,282,955 | 11/1966 | Le Suer.....       | 252/51.5 A |
| 3,373,111 | 3/1968  | Le Suer et al..... | 252/51.5 A |
| 3,390,086 | 6/1968  | O'Halloran.....    | 252/47.5   |
| 3,454,607 | 7/1969  | Le Suer et al..... | 252/47.5 X |
| 3,498,915 | 3/1970  | Coleman.....       | 252/47.5   |
| 2,179,061 | 11/1939 | Smith.....         | 252/406 X  |
| 2,447,619 | 8/1948  | Rogers et al.....  | 252/406 X  |
| 2,732,346 | 1/1956  | Jones et al.....   | 252/45     |

FOREIGN PATENTS OR APPLICATIONS

952,151 3/1964 Great Britain

OTHER PUBLICATIONS

Kalichevsky et al. "Petroleum Refining with Chemicals" (1956) pages 525-534

Primary Examiner—Daniel E. Wyman

Assistant Examiner—W. Cannon

Attorney—Pearlman and Stahl and Ernest V. Haines

[57]

ABSTRACT

Mineral lubricating oil compositions are prepared containing sludge dispersing amounts of conventional ashless dispersants and, optionally, their sulfurized derivatives, and also containing sludge inhibiting or oxidation inhibiting amounts of sulfurized oil-soluble pour point depressant type organic compounds. The ashless dispersants used are the polyalkylene polyamine condensation products of alkenyl succinic acids or anhydrides or of alkenyl substituted lower fatty acids wherein the alkenyl radical is of C<sub>40</sub> to C<sub>25</sub> length used either alone or along with their sulfurized derivatives. The pour point depressants are those heretofore conventionally used but in their sulfurized form, such as sulfurized wave alkylated naphthalene, sulfurized polymeric long chain alkyl esters of acrylic or methacrylic acids.

7 Claims, No Drawings

## LUBRICATING OIL COMPOSITIONS CONTAINING IMPROVED SLUDGE INHIBITING ADDITIVES

The present invention relates to the use in mineral lubricating oil compositions of a combination of oil-soluble sulfurized pour point depressant-type compounds with the so-called ashless dispersants which are likewise oil-soluble and which have been used in lubricating oil compositions for several years. In addition, the additive admixtures may contain sulfurized ashless dispersants of the same or different ashless dispersants used.

Numerous addition agents have heretofore been prepared for use in mineral lubricating oils including the so-called heavy duty oils which are employed in railroad diesel engines and gas engines. Prior researchers have been successful in finding various types of oil-soluble organic compounds which exhibit specialized and specific properties of a beneficial nature when they are incorporated into mineral lubricating oils. For many years now, organic compounds have been added in minor amounts to lubricating oils for the purpose of lowering their pour point, of improving their viscosity index, of affording increased resistance to oxidation, of imparting antiwear properties, of inhibiting sludge formation and of dispersing sludge when it is formed during use of the oils. The use of such additives at the present time enjoys widespread commercial acceptance. Good oxidation stability and good dispersing along with good detergency have become essential requirements for engine lubricating oils. This is particularly so in connection with lubricating oils used in so-called heavy duty engines such as gas engines and railroad diesel engines. Additionally the additives employed must necessarily be accepted from the standpoint of lack of wear or attack on the specialized types of bearings employed in internal combustion engines at the present time. Copper-lead containing bearings are usually susceptible to wear and corrosion and suitable compounded oils must exhibit low corrosion and low bearing wear with respect to such specialized bearings in order to be acceptable commercially.

In the past, it has been proposed to add sulfurized polyisobutylene to lubricating oils. See, for example, Cohen U.S. Pat. No. 2,312,750. Also, it has been proposed in the past to employ sulfurized ashless dispersants in lubricating oils, see British Pat. No. 1,101,040 and U.S. Pat. No. 3,390,086.

By incorporating elemental sulfur into oil-soluble pour-point-depressant-type organic compounds, many of which have been conventionally used heretofore as pour point depressants, it is possible to impart, in addition to the pour point properties, (which are not materially sacrificed) anti-oxidant properties as well, so that even in the case of lubricating oil compositions being subjected to extremely high temperatures during use the combined or dual properties are utilized. It has now been discovered that the tendency of formation of sludge and other deposits in lubricating oils is lessened or minimized by using, in combination in such lubricating oils, at least two additives, namely an ashless dispersant which tends to disperse sludge and to prevent its deposition in the engine and a sulfurized pour point depressant or a sulfurized compound closely akin to such depressants which has anti-oxidant properties and which imparts an initial and added resistance to sludge formation through oxidation inhibition. Such a combination of additives leads to an enhanced elimination of the tendency to form sludge by chemical reduction of the sludge precursors in addition to the usual dispersion of the sludge that is formed. It has been discovered, however, there is a synergistic enhancement of the desired properties in lubricating oils when these two types of materials are used together in a mineral lubricating oil composition.

Although it is not necessary that the pour point depressant types of compounds in and of themselves possess pour point depressant properties when added to lubricating oils, the present invention finds its greatest utility when conventional pour point depressant compounds are subjected to a reaction with elemental sulfur, for it has been discovered that the pour point depressant properties of such compounds which have

been conventionally employed in the past are not destroyed but in addition by the introduction of the elemental sulfur into a chemical bond with such compounds additional properties are imparted to these pour point depressants, namely antioxidant and sludge precursor destroying properties which tend to minimize and decrease the normal tendency of such oils to degradative oxidation and hence sludge formation. Other compounds may be employed, i.e. compounds other than

those which in their unsulfurized form do, in fact, depress the pour point of such mineral lubricating oils. These compounds are referred to as pour point depressant type compounds because their chemical configuration is analogous to the chemical configuration of the compounds which do possess pour point depressant properties and they are homologues or analogues thereof which are oil-soluble. Both types of compounds, i.e. pour depressants and the closely related compounds not possessing pour point depressant properties, are intended to be included in the expression "pour point depressant type compound" or the expression "pour point depressant type organic compound" as used herein and in the claims.

The types or classes of compounds that may be treated with elemental sulfur or its chemical equivalent, i.e. sodium polysulfide, for example, are all oil-soluble and have generally number average molecular weights of between about 900 and about 20,000, preferably between about 1200 and about 10,000. They may be broadly defined in the following classes:

1. long chain  $C_8-C_{30}$  alkylated-benzene, -phenols, -naphthalene, -naphthols, i.e. paraffin-wax-alkylated naphthalene, wax alkylated phenol;

2. long chain ( $C_8-C_{30}$ ) alkylated  $C_1-C_5$  alkyl substituted benzene, naphthalene, phenol, or naphthol compounds, i.e. paraffin-wax-alkylated cresols, wax-alkylated toluene, wax-alkylated alpha or beta methyl naphthalene, wax alkylated 1-methyl beta naphthol, etc.;

3. polymers of  $C_2-C_{28}$  alkyl esters of monoolefinically unsaturated monocarboxylic acids, e.g. acrylic, methacrylic, or vinyl acetic acid esters of butyl, amyl, hexyl, decyl, lauryl, cetyl or stearyl alcohols; polylauryl acrylate, polymers of mixed  $C_{12}-C_{18}$  (Lorol) alcohols esterified with acrylic acid or methacrylic acids;

4. polymers of  $C_6-C_{28}$  dialkyl or dialkenyl esters of alpha-beta unsaturated dibasic carboxylic acids or anhydrides thereof, e.g. maleic or fumaric acid esterified with octyl alcohol or  $C_{8+}$  oxo alcohols, di-Lorol fumarates, didodecyl maleate;

5. polymeric  $C_{20}-C_{22}$  acylated polystyrene, e.g. behenyl polystyrene; acetyl wax alkylated polystyrene;

6. polyacryl amides, i.e. N-vinyl pyrrolidone or N-vinyl pyrrolidone copolymerized with  $C_4-C_{20}$  fatty acids, polymeric N-octadecyl methacrylamide, N-octadecenyl polyethylacrylamides;

7. copolymers of vinyl esters of  $C_2-C_6$  fatty acids, or  $C_4-C_6$  alpha monoolefins, with monomers of (4) i.e. di  $C_6-C_{28}$  dialkyl esters of alpha, beta unsaturated dicarboxylic acids or anhydrides; copolymers of di-Lorol ( $C_{12}-C_{18}$ ) fumarate with vinyl acetate, copolymers of di  $C_{28}$  alkyl fumarate with isobutylene.

All of the above-mentioned classes of compounds are old compositions, most of which have heretofore been used in automotive and marine engines as additives in crankcase lubricants. Their sulfurized derivatives are the novel additives in such crankcase lubricants as described, supra. Various U.S. patents described the methods of preparation and the lubricating oil additive usage of these unsulfurized compounds, for example, group (1) and (2) compounds have been used for many years as pour point depressants as exemplified by the disclosures of U.S. Pat. Nos. 1,815,022; 2,015,748; 2,087,682; 2,174,246 and 2,191,498; group (3) compounds by U.S. Pat. Nos. 2,100,993; 2,125,885 and 2,628,225; group (4) compounds by U.S. Pat. No. 2,618,602; group (5) compounds by U.S. Pat. Nos. 2,703,817 and 3,248,186; group (6) compounds by U.S. Pat. No. 2,387,501 and group (7) compounds by U.S. Patents Nos. 2,666,746; 2,721,877; 2,721,878;

2,694,685; 2,825,717 and Reissue 26,134, which disclosures are incorporated herein by reference. No real need is seen for duplicating the description of the usage of the unsulfurized pour point depressants in lubricating oils, herein, nor for duplicating, herein, their methods of production, since they are well known; they have become commercialized and widely marketed additives for their pour point depressant effects and have now been so used for many years. The starting materials, i.e. the materials to be sulfurized in accordance with the present invention are old and widely available on the commercial market.

The pour point depressant type organic compounds are subjected to reaction with elemental sulfur in order to chemically combine the sulfur into the compound. The elemental sulfur or its chemical equivalent, for example, sodium polysulfide, is added in the required amounts and the reacting mixture is maintained at a temperature between about 100° and 260° C., preferably between about 120° and 250° C. for a period of time ranging between about 30 minutes and 40 hours, preferably for between about 4 and about 12 hours. The relative amount of elemental sulfur employed per mole of pour point dispersant type organic compounds used may vary considerably but is generally between about 2 and about 0.5 mole of sulfur, preferably between about 1 and about 0.5 mole of sulfur per mole of organic compound to be sulfurized. The final product will contain sulfur to the extent of between about 1.0 and about 10.0 wt. percent, preferably between about 1.5 and about 7.5 wt. percent sulfur. The sulfurization reaction is preferably carried out in the liquid phase. A particularly convenient liquid reaction medium has been found to be a mineral lubricating oil for the reason that the sulfurized product upon completion of the sulfurization reaction is present in the lubricating oil to the extent of some 50-80 wt. percent and so the entire reaction mixture once it has been purged of hydrogen sulfide by sweeping with nitrogen or other inert gas is suitable for use as an oil concentrate. A typical oil base that has been used as a carrier for the reaction is a solvent extracted neutral lubricating oil of 150 SUS at 100° F. To some extent this oil also is sulfurized but its small amount of sulfurization is not beneficial, per se. The ashless dispersant with or without the addition of sulfurized ashless dispersant may be added to this concentrate. When a lubricating oil concentrate of the sulfurized pour point type organic compound is finally produced or is compounded, the oil-soluble ashless dispersant as well as the sulfurized ashless dispersant, if used, may be added as such or it may be added in the form of a similar solvent neutral 150 SUS base lubricating oil concentrate of from 50-80 wt. percent active ingredient concentration. The amount of the sulfurized pour depressant type organic compound, the amount of the oil-soluble ashless dispersant and the amount of the sulfurized ashless dispersant finally employed in a lubricating oil composition may vary considerably. Suffice it to say that these concentrations are sufficiently large to impart sludge inhibiting, dispersing and/or antioxidant properties to the lubricating oil. The amount involved so far as the upper limit is concerned, is relatively immaterial so long as the minimum effective amount is employed. For practical purposes, all three types of additives are each employed (when employed) in an amount ranging from 0.05 to 10.0 wt. percent based on the total oil composition, preferably between about 0.1 and about 5.0 wt. percent on the same basis.

The oil-soluble ashless dispersants employed are those conventionally employed in lubricating oil compositions. In general, they are formed by a condensation of at least one polyalkylene polyamine with at least one of the following: alkenyl succinic acid, alkenyl succinic anhydride, alkenyl substituted lower fatty acid, wherein the alkenyl group contains from about 40 to about 250 carbon atoms per alkenyl radical. Also, the sulfurized derivatives of such oil-soluble ashless dispersant may be used as before stated and as heretofore referred to as being disclosed in British Pat. No. 1,101,040 and U.S. Pat. No. 3,390,086. These patents not only disclose the production of the sulfurized ashless dispersants of the type

herein contemplated for use but also disclose several methods of preparing the unsulfurized ashless dispersants of the polyalkylene polyamine-alkenyl succinic anhydride or alkenyl fatty acid condensation type. The disclosure of U.S. Pat. No. 3,390,086 is incorporated herein by reference not only as to the sulfurized dispersants but also to lend support and basis for the preparation and use of the unsulfurized ashless dispersants therein disclosed. The Anderson patents and the LeSuer U.S. Pat. Nos. 3,185,646; 3,185,647; 3,200,107 and 3,216,936 are also incorporated herein by reference. They show the preparation and use of these unsulfurized ashless dispersants. The number average molecular weight of the ashless dispersants will generally be between about 700 and about 5,000, preferably between about 800 and about 2,000 and preferably the alkenyl radical constitutes a polyisobutylene or a polypropylene having the requisite 40-250 carbon atoms per radical. An example of a suitable alkenyl lower fatty acid which is condensed with a polyalkylene polyamine is polyisobutetyl propionic acid. This is formed by halogenating the polyisobutylene and condensing it with acrylic acid or an analog, such as alpha methylacrylic acid, crotonic or isocrotonic acid. The polyisobutetyl succinic anhydride or polyisobutetyl succinic acid is obtained conventionally by condensing the polyisobutylene or chloropolyisobutylene with maleic or fumaric acids or maleic anhydride.

The polyalkylene polyamines which are reacted with the carboxylic acids or their anhydrides encompass a considerable number of compounds and are fully described under the heading "Ethylene Amines" in Encyclopedia of Chemical Technology, Kirk & Othmer, Volume 5, pages 898-905 (1950). Any number of specific polyethylene polyamines are available in commerce and marketed. A preferred polyamine which is widely used in preparing the ashless dispersant type condensation products is tetraethylenepentamine. One method of preparing the condensation products of, for example, polyisobutetyl succinic anhydride and tetraethylene-pentamine is disclosed in U.S. Pat. No. 3,172,892 and this material is the material which has been used as the ashless dispersant additives in the hereinafter described specific examples.

The lubricating oils employed as the base oils are preferably mineral lubricating oils which may be derived from naphthenic, paraffinic, aromatic, or mixed crude oils. Generally they will have a viscosity at 210° F. of between about 45 and about 90 SUS (Saybolt Universal Seconds) and at 100° F. a viscosity of between about 150 and about 1,100 SUS. The viscosity indices of these oils will generally range between about 0 and about 100. In the case of oils employed in high speed, heavy duty diesel engines, oils of high viscosity indices are often preferred, i.e. of the order of 100 or higher. Usually most diesel engines employ lubricating oils having viscosities of between about 75 and about 80 SUS at 210° F. and at 100° F. of between about 800 and about 1,250 SUS, with viscosity indices ranging between about 55 and about 80.

Amounts similar to the amounts specified for the novel additives are likewise employed for the conventional additives which are also used in such lubricating oils. These additives are corrosion inhibitors, (sorbitan mono-oleate), antioxidants, (N-phenyl alpha naphthylamine) pour point depressants, (unsulfurized wax alkylated naphthalene), viscosity index improvers (unsulfurized polyisobutylene or polymethyl methacrylates), antiwear agents (the zinc salt of di (C<sub>4</sub>-C<sub>5</sub> alkyl) dithiophosphate), detergents (the alka-line earth metal salts of alkyl substituted phenol thioethers or sulfides), and dispersants (alkaline earth metal salts of petroleum sulfonic acids or of alkaryl sulfonic acids and the like).

The following examples are illustrative of the character and nature of the invention but it is not intended that the invention be limited thereto.

#### EXAMPLE 1

About 400 grams of paraffin wax alkylated naphthalene, which is conventionally employed as a pour point depressant

for lubricating oils, was reacted with about 8 grams of sulfur at a temperature of 180°C. (356°F.) for 7 hours. After filtration of the product, the filtrate analyzed about 1.42 wt. percent of sulfur.

The resultant material and the starting material were both subjected to a series of comparative sludge inhibition tests in which the base oil composition involved the use of a sludge-containing used oil which was freed of solid sludge by centrifuging for one hour at 1,800 rpm. Ten grams of the supernatant oil freed of solid sludge particles, but containing oil-soluble sludge precursors, was employed as the base oil in this test. The oil, without any further additives, upon heating to the temperature applied in the test, would tend to form additional oil-insoluble deposits of sludge. In a tared stainless steel centrifuge tube, 10 grams of the supernatant used oil containing 1.0 wt. percent of the additive to be tested with or without 0.4 wt. percent of an ashless dispersant was heated to 150°C. (300°F.) for 2 hours in a constant temperature oil bath. Following the heating, the tube was cooled and then centrifuged for one hour at 1,800 rpm. The supernatant oil was decanted again from the tube and any residual sludge deposits were washed carefully with 99 percent n-pentane to remove all remaining oil associated therewith. The weight of the solid sludge formed during the test was determined. Blank or other comparative runs were also carried out in which either no additive was employed or an additive, to be compared, was employed. A substantial decrease in the amount of sludge deposited, as compared with the amount deposited in the case of the blank run, indicates the extent, if any, that the additives had a sludge inhibition effect, through the actual measurement, in milligrams, of the weight of the sludge formed. The following comparative data were obtained:

TABLE I

| Run No. |                                                                             | Sludge, Milligrams<br>Per 10 Grams Used<br>Oil |
|---------|-----------------------------------------------------------------------------|------------------------------------------------|
| A       | 1 wt. % wax alkylated naphthalene (molecular weight about 1000)             | 11.2                                           |
| B       | 1 wt. % sulfurized wax alkylated naphthalene                                | 11.1                                           |
| C       | 1 wt. % sulfurized wax alkylated naphthalene plus 0.4% ashless dispersant   | 7.0                                            |
| D       | 1 wt. % unsulfurized wax alkylated naphthalene plus 0.4% ashless dispersant | 8.5                                            |
| E       | 0.4% ashless dispersant (alone)                                             | 8.0                                            |
| F       | 1 wt. % sulfurized solvent neutral 150 SUS at 100°F. oil                    | 16.5                                           |
| G       | 1 wt. % unsulfurized solvent neutral 150 SUS at 100°F. oil                  | 12.8                                           |

Note: Run F additive was prepared by reacting the unsulfurized solvent 150 neutral oil (400 grams) with elemental sulfur (16 grams) at 180°C. for 10 hours and stripping the reacted mixture with nitrogen at 120°C. for 1 hour. The product analyzed 1.42 wt. percent of sulfur. The blank used oil showed 10.5 mg. of sludge per 10 grams of oil.

It is apparent from these data that the use of sulfurized wax alkylated naphthalene in combination with the ashless dispersant which is identified as being formed by condensing polyisobutylene succinic anhydride with tetraethylenepentamine as disclosed in U.S. Pat. No. 3,172,892 (a conventionally marketed and commercially available ashless dispersant) resulted in the production of less sludge under the conditions of testing than did the use of any other combination of sulfurized or unsulfurized materials with or without the presence of the ashless dispersant.

## EXAMPLE 2

150 grams of the copolymer of di-Lorol fumarate and vinyl acetate as a 50 percent concentrate in solvent neutral 150

70

75

mineral lubricating oil having molecular weights of about 10,000 (this can vary between 8000 and 12,000) was reacted with 7.5 grams of elemental sulfur at a temperature of 180°C. for about 6 1/2 hours. The unreacted sulfur was removed from the reacted mixture by filtration. The filtrated product had a combined sulfur content of about 1.75 wt. percent.

The sludge inhibition test described in Example 1 was carried out using the same used oil containing sludge precursors as was employed to secure the data in Table I. The used oil containing 1 percent of the sulfurized product of Example 2 showed a sludge formation of 7.1 mg. per 10 grams of used oil while the used oil containing no sulfurized product showed the formation of 10.5 mgs. of sludge per 10 grams of used oil.

15

## EXAMPLE 3

150 grams, as a 60 percent concentrate in lubricating oil, of a polymer of the ester formed by esterifying a mixture of methacrylic acid with a mixed C<sub>12</sub>—C<sub>18</sub> alcohol fraction and having the molecular weight of about 10,000 was sulfurized with 7.5 grams of elemental sulfur at a temperature of 180°C. for about 6.5 hours. The unreacted sulfur was removed by filtration and the filtrate had a combined sulfur content of 1.73 wt. percent.

20 25 The same sludge inhibition test on used oil, as described in Example 1, was undertaken on a comparative basis with and without the presence of a conventional ashless dispersant. The comparative data are as follows:

30

TABLE II

| Run No. | Sludge, Milligrams<br>Per 10 Grams Used<br>Oil                             |
|---------|----------------------------------------------------------------------------|
| H       | 1% product of Example 3                                                    |
| I       | 1% unsulfurized polymer of Example 3                                       |
| J       | 3% sulfurized product of Example 3                                         |
| K       | 3% unsulfurized polymer starting material of Example 3                     |
| L       | 1% sulfurized polymer of Example 3 plus 0.4% ashless dispersant            |
| M       | 1% unsulfurized reactant polymer of Example 3 plus 0.4% ashless dispersant |
| N       | 0.4% ashless dispersant (no additives)                                     |
| O       |                                                                            |

50 55 Note: The ashless dispersant employed was the same ashless dispersant as shown in Table I, i.e. the condensation product of polyisobutylene succinic anhydride with tetraethylenepentamine and was used as a 70 percent concentrate in mineral lubricating oil in securing the data in Table I.

## EXAMPLE 4

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 86

|   |                                                                            |      |
|---|----------------------------------------------------------------------------|------|
| Q | 1% unsulfurized reactant polymer of Example 4                              | 56.6 |
| R | 1% sulfurized product of Example 4 plus 0.4% ashless dispersant            | 5.2  |
| S | 1% unsulfurized reactant polymer of Example 4 plus 0.4% ashless dispersant | 11.3 |
| T | 0.4% ashless dispersant (no additives)                                     | 8.0  |
| U |                                                                            | 22.0 |

Note: the same ashless dispersant as described in Tables I and II was employed in securing the data appearing in Table III.

It is apparent from the study of the comparative data appearing in Tables II and III that the combination of using an ashless dispersant together with a sulfurized polymeric material having a sufficiently high molecular weight to impart oil solubility and having a structural configuration so as to give, in unsulfurized form, a pour point depressant effect gives unexpected oxidation-inhibition when used in mineral lubricating oils which normally have a tendency to form sludge.

What is desired to be secured by Letters Patent is:

What is claimed is:

1. A lubricating oil composition comprising a major proportion of a mineral lubricating oil,

a minor sludge inhibiting amount of a sulfurized polymeric  $C_6$  to  $C_{28}$  alkyl ester of acrylic or methacrylic acid, said ester having lubricating oil pour point depressant properties, said sulfurized ester containing about 1 to 10 wt. per-

cent of sulfur, and a minor sludge dispersing amount of at least one oil-soluble ashless sludge dispersant selected from the group consisting of condensation products of polyalkylene polyamines with alkenyl succinic acid, alkenyl succinic anhydride, and alkenyl propionic acid, wherein the alkenyl radical has from about 40 to 250 carbon atoms.

2. A lubricating oil composition as defined by claim 1 wherein said sulfurized ester and said ashless dispersant are each present in a concentration between about 0.05 and about 10 wt. percent of the total composition.

3. A lubricating oil composition as defined by claim 1 which also contains a minor sludge inhibiting amount of at least one sulfurized ashless dispersant wherein said ashless dispersant is as set forth in claim 1.

4. A lubricating oil composition as defined by claim 1 wherein said sulfurized polymeric ester is a sulfurized polymeric mixed  $C_{12}$ — $C_{18}$  alkyl methacrylate.

5. A lubricating oil composition as defined by claim 1 wherein said polyalkylene polyamine is tetraethylene pentamine.

6. A lubricating oil composition as defined by claim 1 wherein said alkenyl radical is polyisobutylene.

7. A lubricating oil composition as defined by claim 1 wherein said ashless dispersant is the condensation product of tetraethylene pentamine and polyisobutylene succinic anhydride.

\* \* \* \* \*

30

35

40

45

50

55

60

65

70

75